

**1****3,376,107****STOICHIOMETRIC TRANSITION  
METAL HYDRIDES**Akira Oka, 71 Sugamo 1-chome, Toshima-ku,  
Tokyo, JapanNo Drawing. Filed May 15, 1964, Ser. No. 367,843  
Claims priority, application Japan, May 20, 1963,  
38/25,289; Oct. 10, 1963, 38/52,715; Jan. 31,  
1964, 39/4,410; Feb. 18, 1964, 39/8,362; Feb.  
21, 1964, 39/9,028

1 Claim. (Cl. 23—204)

**ABSTRACT OF THE DISCLOSURE**

This invention relates to stable stoichiometric hydrides of metals of IV-B group of the periodic table and preparation method thereof and utilization thereof in the powder metallurgical process.

The object of this invention is to provide a rapid and economical process of producing stable stoichiometric IV-B metal hydrides.

One utilization of this invention is to provide an ultra-fine powder of IV-B metal hydrides and IV-B metals.

Another utilization of this invention is to provide a simple and economical method of producing an non-porous sintered metal.

Another utilization of this invention is to provide a process for preparing single crystals of transition metals.

Another utilization of this invention is to provide a rapid and economical method of producing non-porous sintered alloys of varying compositions.

Another utilization of this invention is to provide chemically inert metallic receptacles by the process of depositing a stable IV-B metal on the surface of less expensive metals.

Another utilization of this invention is to provide a simple methods to prepare cermets of any IV-B metal.

The success of this invention depends upon a new theory concerning the phenomenon that stoichiometric transition metal hydrides exist in a state which is very stable against air oxidation at room temperature, and they behave differently from powdered metals in the sintering process. Metallic bonding of great strength acts between activated titanium atoms produced by thermal decomposition of metallic hydrides, and a non-porous sintered material is obtained. On the other hand, in a case of ordinary powder metallurgical process using metal powder, a sintering process is interfered with a thin oxide film on a surface of the metal powder.

The published literature concerning the IV-B metal hydrides does not provide very precise information concerning their true structure. For instance, Moellor stated in his "Inorganic Chemistry," "The quantity of hydrogen present ordinarily bears no exact stoichiometric relation to the metal, and formulas such as  $TiH_{1.72}$  and  $TaH_{0.68}$  which are often given, probably represent no more than the conditions essential to saturation of the metal with hydrogen." R. P. Gibb stated in his paper (J. Electrochem. Soc. 93 198 (1948) "Transition metal hydrides are structural complexities between intermetallic and interstitial compound." Hansen summarised the available information concerning titanium hydride, and stated, "There is complicating experimental evidence whether the homogeneity range of  $\gamma$  phase extends nearly or wholly up to the composition  $TiH_2$ , or whether even a distinct  $TiH_2$  exists. R. P. Gibb and W. Kruschwitz claimed the preparation of stoichiometric  $TiH_2$  which they report to be unstable below 400° C." And Gibb stated, "Whether this limiting composition is properly called a compound

**2**

is debatable. There is unequivocal evidence that its composition and gross properties are definite and reproducible and that its X-ray diffraction pattern contains moderately strong lines not hitherto reported in the titanium-hydrogen system. These novel lines are two in number ( $d=2.076$  Å, 1.801 Å) and are observable only for freshly prepared materials and are found to disappear gradually as the hydride is stored over a period of a few weeks in air."

10 The titanium, zirconium, hafnium hydride which the inventor prepared by heating high purity commercial sponge titanium, zirconium, hafnium with high purity hydrogen, obtained by passing the hydrogen through a Pd alloy membrane (U.S.P. 2,773,561) at atmospheric pressure is stoichiometric in composition and stable in air. The X-ray diffraction pattern showed no change over a two week period after it was produced. Titanium hydride which was powdered under atmospheric conditions in a mechanical agate mortar did not change its 15 X-ray diffraction pattern except that some line broadening occurred. Stoichiometric titanium hydride is not pyrophoric although, it was found that the powdered titanium metal produced by thermal decomposition of the titanium hydride at 500° C. and a pressure of  $10^{-3}$  mm. 20 Hg is strongly pyrophoric. So fine powder of titanium hydride thus obtained is more stable against air oxidation than fine powder of metal.

The hydrogenation process was accomplished in a few minutes at atmospheric pressure in contrast to the commercial process which is carried out at low pressure for a period of 30 hours.

The stability against air oxidation of stoichiometric titanium hydride and the activated state of the metal produced by thermal decomposition of the hydride and 35 sintering of the resultant titanium metal powder, make it possible to produce high grade titanium metal without the necessity of heating titanium to its melting point.

Many powdered metals have oxide surface which interferes with the sintering process. Stoichiometric IV-B 40 metal hydrides are not subject to this source of interference and when thermal decomposition in vacuo occurs, titanium atom combines each other by excellent metallic bonding, and a sintered specimen is obtained.

Upon annealing this specimen, microcrystalline of titanium is produced which grows to a large single crystal.

All of the above-mentioned characteristics of stoichiometric IV-B metal hydrides make it possible to prepare non-porous alloys of varying composition without the necessity of melting any of the components of the 50 alloys.

Fine powders of transition metal hydrides were mixed, pressed and moulded. After dehydrogenation at temperature higher than 500° C. at a pressure of  $5 \times 10^{-5}$  mm. Hg, the specimen was heated at sintering temperature for two hours, and a non-porous alloy was obtained. When a mixture of hydride powder and metal powder were treated similarly, a non-porous alloy was also obtained. Metal hydrides at high temperatures have a strong reducing power which causes reduction of oxide film of 55 metal surface.

All of the above mentioned factors make it possible to apply titanium and other IV-B metals as coating on steel surface. A fine powder of titanium and 5% of camphor by weight were dispersed in methyl alcohol and the suspension was painted or sprayed on a clean surface of steel. After thermal decomposition in vacuo, it is heated at 60 1200° C. for 3 hours, and a complete non-porous coating of titanium was obtained.

This specimen was unaffected when kept in contact with 0.5 N HCl for two days. A tantalum coating prepared in the same manner was unaffected when kept in contact with 2 N HCl for two days. Chemical apparatuses

for handling acid solution can thus be economically fabricated. Titanium is chemically stable against sea water, so titanium-coated steel pipe can be safely used in contact with sea water.

In addition to all of the above-mentioned factors, a nature of fine powder of stoichiometric transition metal hydride to make a eutectic with a metal surface, make it possible to bond materials. Steel and copper can adhere by a thin paste of titanium hydride at 950° C.

Cermets can combine using stoichiometric IV-B metal hydride without melting any component of the system. This fact can compare with an ordinary bonding using cobalt, which melts upon sintering.

#### EXAMPLE 1

Preparation of stoichiometric IV-B metal hydride. About 5-10 g. of a commercial purity sponge titanium (99.9%), was outgassed by heating at 800° C. under vacuum of  $5 \times 10^{-5}$  mm. Hg, then cooled to 450° C. and a high purity hydrogen, obtained by passing the hydrogen through a Pd alloy membrane (dew point -70° C.) at one atmospheric pressure. (U.S.P. 2,773,561.) Hydrogenation was finished within a few minutes. The composition of titanium hydride was determined by gravimetric analysis, and the mean value of 20 experiments was  $TiH_{1.9982} \pm 0.0063$ . An ordinary analytical method by an ignition showed the same data (4.04% H) with this gravimetric analysis. Utilizing the same process in the case of zirconium sponge (99.6% Zr)  $ZrH_{1.9994} \pm 0.0022$  and with hafnium sponge (99.3% Hf + Zr),

$$HfH_{2.018} \pm 0.025$$

were obtained. Larger quantity of hydrides was prepared as follows. About 150 g. of commercial purity sponge titanium (99.9%) was outgassed in the same manner as above. Using a hydrogen purifier of 1 m.<sup>3</sup> hour capacity, and stoichiometric titanium hydride was obtained.

#### EXAMPLE 2

Production of stoichiometric titanium hydride using titanium as a gettering agent for the purificaton of hydrogen.

Sponge titanium was heated higher than 850° C. in vacuo and cylinder hydrogen was passed over a layer of sponge titanium (-10 mesh), which absorbed impurities in hydrogen (water vapour, oxygen, and nitrogen), and another layer of sponge titanium which was situated some distance under the gettering titanium layer absorbed purified hydrogen to form hydride of a stoichiometric composition.

The stoichiometric IV-B metal hydrides obtained by the above examples had the same FCC X-ray diffraction pattern, and the X-ray diffraction pattern did not change over a period of several weeks as did the X-ray diffraction pattern of R. P. Gibb as mentioned earlier. It is, therefore, true that this is the first preparation of a stable stoichiometric IV-B metal hydride.

#### EXAMPLE 3

Preparation of fine powder of stoichiometric IV-B metal hydrides and fine powder of said metals.

Powder of stoichiometric titanium hydride was obtained from the stoichiometric titanium hydride produced by the above-mentioned process by pulverizing it with a mechanical agate mortar for a week. During this process colloidal fine particles entered atmosphere and were collected by an electric precipitator. Such fine powder has been made by the invention for the first time.

The above-mentioned fine powder of stoichiometric titanium hydride was heated higher than 500° C. in a vacuum of  $5 \times 10^{-5}$  mm. Hg, and a fine powder of titanium was obtained. This titanium powder is pyrophoric.

#### EXAMPLE 4

Preparation of a non-porous sintered specimen.

Stoichiometric titanium hydride, of a mean diameter

of  $3\mu$  was pressed into a plate of 11.3 mm. diameter under a pressure of 5 tons/cm.<sup>2</sup>. It was then heated higher than its decomposition temperature under a vacuum of  $5 \times 10^{-5}$  mm. Hg. Then the activated titanium was sintered at 1200° C. for 2 hours and allowed to cool. The sintered plate which was prepared by this process had no porosity and its density was 4.52 approximately. This is the first non-porous sintered titanium.

#### EXAMPLE 5

Preparation of a single crystal of titanium.

Using the powder of titanium hydride prepared as above, a plate of 50 x 25 x 3 mm. was prepared using the same pressure, and the non-porous plate was obtained by the same sintering process which was shown to be microcrystalline titanium. After annealing process at 1250° C. for 2.5 hours and cooling over a night, it was revealed that the plate consisted of 4 single crystals of titanium.

#### EXAMPLE 6

Preparation of non-porous alloys by sintering of stoichiometric metal hydrides.

Mixed 0.6 g. of fine powder of stoichiometric titanium hydride and 0.6 g. of fine powder of stoichiometric zirconium hydride with an agate mortar for one hour. Pressed into a pellet of 11.3 mm. diameter by a pressure of 6 tons/cm.<sup>2</sup>. Dehydrogenated in a vacuum of  $10^{-6}$  mm. Hg at 800° C. Sintered at 1250° C. for 2 hours. And a non-porous alloy was obtained.

#### EXAMPLE 7

Preparation of alloys by sintering of stoichiometric IVb metal hydride and metal powder.

One gram (1 g.) of fine powder of stoichiometric zirconium hydride and 0.2 g. of molybdenum powder (-200 mesh) were mixed by an agate mortar. The mixture was treated in the same manner as in Example 6, and a non-porous alloy was obtained.

#### EXAMPLE 8

Metal coating prepared by using stoichiometric titanium hydride and tantalum hydride.

The fine powder of titanium hydride mentioned above was dispersed in methyl alcohol containing camphor and painted on a clear surface of a steel rod (carbon content 0.15%). The rod was then heated in vacuo higher than 500° C. for dehydrogenation. The rod was then heated at 1200° C. for 3 hours under a vacuum of  $5 \times 10^{-5}$  mm. Hg. A titanium-coated steel rod was obtained. The rod was immersed in 0.5 N HCl for two days, no effect on the rod was noted, while an identical steel rod without coating which was immersed in the same solution lost 50 mg. in weight.

#### EXAMPLE 9

Adhesion of metals using stoichiometric titanium hydride.

A sandwich arrangement was made by a plate of stainless steel, a thin paste of titanium hydride powder dispersed in methyl alcohol and a plate of copper. This specimen was pressed by a clamp, then heated at 950° C. under a vacuum of  $5 \times 10^{-5}$  mm. Hg for 2 hours, and an excellent bond which showed no change upon strong heating with a gas burner was obtained.

#### EXAMPLE 10

Preparation of cermets using stoichiometric titanium hydride. Mixed 0.5 g. tungsten carbide and 0.5 g. of fine powder of stoichiometric titanium hydride with an agate mortar, pressed into a pellet of 11.3 mm. diameter by a pressure of 5 tons/cm.<sup>2</sup>. Dehydrogenated in a vacuum of

$5 \times 10^{-5}$  mm. Hg at 600° C., sintered at 1200° C. for an hour. And a sintered piece is obtained without melting any component of the pellet.

What I claim is:

1. Process for preparing stable metal hydrides of metals of Group IV-B having the general formula  $\text{MeH}_2$ , where Me stands for a IV-B metal comprising the steps of:
  - (I) purifying hydrogen by passing it thru a Pd alloy membrane with a dew point of -70° C. at one atmosphere pressure to obtain high purity hydrogen;
  - (II) providing in a reaction zone a high purity sponge metal of -10 mesh selected from the group consisting of Ti at 99.99%, Zr at 99.6%, and Hf at 99.3%, said sponge being divided into a first gettering layer and a second layer spaced from and underneath said gettering layer;
  - (III) outgassing said sponge metal by heating it to at least 800° C. under a vacuum;
  - (IV) cooling said sponge metal heated by the previous step to about 450° C. while maintaining the vacuum;
  - (V) directing said purified hydrogen thru said sponge metal in the reaction zone while maintaining said atmospheric pressure and the temperature of about 450° C., whereby the first layer absorbs gaseous impurities from the hydrogen and the purified hydrogen emerging therefrom passes thru the second layer to form a stable stoichiometric hydride: of titanium, having a formula in the range of  $\text{TiH}_{1.9982 \pm 0.0063}$ .
2. of zirconium, having a formula in the range of  $\text{ZrH}_{1.994 \pm 0.0022}$ .
3. and of hafnium, having a formula in the range of  $\text{HfH}_{2.018 \pm 0.025}$ .

### References Cited

#### UNITED STATES PATENTS

|           |         |                      |          |
|-----------|---------|----------------------|----------|
| 1,816,830 | 8/1931  | Driggs -----         | 23-204 X |
| 2,452,139 | 10/1948 | Newton -----         |          |
| 2,536,610 | 1/1951  | King et al. -----    | 23-210 X |
| 3,152,868 | 10/1964 | Kempter et al. ----- | 23-204   |
| 1,120,561 | 12/1914 | Strong et al. -----  | 55-2     |
| 2,495,761 | 1/1950  | Platt -----          | 156-157  |
| 2,994,606 | 8/1961  | Goodzeit -----       | 75-214   |
| 3,072,499 | 1/1963  | Cole et al. -----    | 117-130  |
| 3,107,175 | 10/1963 | Cape -----           | 117-130  |
| 3,111,441 | 11/1963 | Grundel -----        | 156-157  |
| 3,116,112 | 12/1963 | Jenkner -----        | 23-204   |
| 3,144,357 | 8/1964  | Hulme et al. -----   | 148-1.6  |
| 3,150,975 | 9/1964  | Beaver et al. -----  | 75-214   |
| 3,152,868 | 10/1964 | Kempter et al. ----- | 23-204   |
| 3,165,397 | 1/1965  | Lobo -----           | 75-0.5   |
| 3,186,829 | 6/1965  | Landgraf -----       | 75-0.5   |
| 3,186,880 | 6/1965  | Skaggs et al. -----  | 148-1.6  |

#### OTHER REFERENCES

Ellis, "Hydrogenation of Organic Substances," 3rd edition, 1930, p. 862.

Hurd, "Chemistry of the Hydrides," 1952, pp. 181-184.

Pascal, "Noveau Traite DeChime Minerale," January 1963, vol. 9, pp. 172-175, 447-457, 938-944.

MILTON WEISSMAN, *Primary Examiner.*

LEON D. ROSDOL, OSCAR R. VERTIZ, *Examiners.*

R. L. GRUDZIECKI, *Assistant Examiner.*